

May 23, 1961

N. E. STONE

2,985,855

COATING FOR SHEET STEEL IN TRANSFORMER CORES

Filed Jan. 11, 1957



Inventor  
Norman E. Stone  
By Houston L. Swanson  
Attorney

1

2,985,855

**COATING FOR SHEET STEEL IN  
TRANSFORMER CORES**

Norman E. Stone, Pittsburgh, Pa., assignor to Allis-Chalmers Manufacturing Company, Milwaukee, Wis.

Filed Jan. 11, 1957, Ser. No. 633,664

2 Claims. (Cl. 336—60)

This invention relates in general to wound magnetic cores and in particular to wound magnetic cores provided with an insulating and spacing coating of a predetermined form.

Electrical steel is sometimes supplied to the transformer manufacturer in either a semifinished state or a fully processed state in the form of large sheets or rolls. After the material is processed to a size convenient for the core manufacturing process it is given a high temperature anneal in the case of the semifinished state which results in crystal growth in the preferred direction, further purification of the steel and in the case of the fully processed state, a low temperature anneal which results in relief of any strains set up in the material during the manufacturing process. During the annealing process the magnetic steel material is in the form of a coil or rolled strip. Thus, there is relatively large surface contact between the layers of the magnetic material while in the annealing furnace. Due to the plasticity of the steel at the elevated temperatures associated with the recrystallization anneal, there is a tendency for the associated layers in the assembly to stick together and possibly even weld to one another. It, therefore, becomes desirable to have a coating with a refractory substance between adjacent layers during the high temperature anneal to avoid this sticking, and which will also provide an insulating coating.

It often becomes necessary, during the process of manufacturing wound cores to unwind the annealed rolled strip and wind it around the winding leg of a preformed coil winding. To facilitate this step, it is usually desirable to have a slight degree of spacing between the layers of the wound core prior to annealing it.

In other methods of making wound cores, this spacing is formed by inserting shims or spacing elements between the layers prior to annealing. Paper, thread, and other carbon elements have been used as spacing elements. These materials burn or char at the annealing temperatures and the carbon thus formed contaminates the annealers. Consequently, the annealers must be frequently cleaned. In addition, these carbon spacers are limited to use in low temperature stress annealing. If used in high temperature recrystallization annealing, the carbon migrates to the wound steel material and defeats the purpose of the recrystallization annealing.

Wire has also been used as a spacer but has not produced a uniform degree of spacing and has frequently resulted in grooves in the rolled steel strip. During high temperature annealing the wire frequently fused with the steel strip.

Increasing the thickness of the insulating coating on the steel strip to act as a spacer has also been attempted. However, when building up large quantities of the coating there is less probability of obtaining a uniform degree of spacing between the laminations of the wound steel strip. Because of the increased area of the coating providing the spacing it is extremely difficult to obtain a uniform coating surface. Thus a spacer of a noncarbon substance which

2

will not adversely affect the steel strip and which will provide a uniform degree of spacing will overcome the aforementioned objections.

According to this invention such a uniform degree of spacing between the laminations of the wound steel strip is obtained by covering the strip with a coating comprising a refractory substance and a bonding agent. The exposed surface of this insulating coating is formed into raised areas of spacing elements or spacers.

According to the present invention the insulating coating with spacers can be applied to the top and bottom surfaces of the magnetic sheet material by applying the coating substance to the surfaces and forming this substance into predetermined positioned high areas of spacing elements.

It is therefore an object of this invention to provide a magnetic sheet material with an insulating coating having raised areas.

A further object of this invention is to provide a wound core having a uniform predetermined space between laminations.

A still further object of this invention is to provide a wound core with removable spacing elements.

Another object of this invention is to provide an improved method of building wound cores with predetermined spacers between the laminations in the core.

Objects and advantages other than those mentioned above will be apparent from the following description:

Fig. 1 is a schematic view illustrating the process of coating a magnetic sheet material for wound cores;

Fig. 2 is an isometric view of a grooved roll;

Fig. 3 is a top view of magnetic sheet material with an insulating coating having spacers; and

Fig. 4 is an enlarged cross sectional view of Fig. 3 on line IV—IV.

In accordance with the present invention, magnetic sheet material or a silicon steel strip 11 is covered preferably on both top and bottom surfaces with an adherent coating solution 12 thereon. This coating contains a finely divided refractory substance, a bonding agent, and water.

Any known refractory substance such as lime, dolomite, magnesium oxide and silica, and various combinations of the above may be used. A preferred bonding agent is carboxymethyl hydroxyethyl cellulose sold by the Hercules Powder Company under the name of CMHEC. However, this invention is not limited to carboxymethyl hydroxyethyl cellulose as other bonding agents such as methyl cellulose, and an alkyd resin or cellulose acetate in suitable organic solvents may be used.

A preferred coating solution 12 may be prepared by adding 175 pounds of refractory substance, a mixture of calcium oxide and magnesium oxide, 325 mesh, and 16.7 pounds of carboxymethyl hydroxyethyl cellulose to a sufficient amount of water to form a slurry. These ingredients are then ground in a wet ball mill for several hours until the refractory particles are thoroughly dispersed. It has been found that a suitable coating is obtained when the specific gravity of the solution is substantially 1.07 and its viscosity is 18.5 in a .2 Zahn cup.

The coating solution 12 is then ready to be applied to the top and bottom broad surfaces of the sheet material 11. The resulting unsymmetrical exposed surface of the coating is then formed into relatively high and low areas forming an insulating coating 21 with two different thicknesses. The raised areas 22 are of a uniform height with a predetermined cross section and serve as spacing elements.

The sheet material 11 with its adherent insulating coating 21 is then placed in an oven 16 where evaporation of the excess fluid in the coating occurs. As a result of evaporation the coating is transformed into a solid

form. The surface of the coating adjacent the sheet material remains adherent and the exposed surface of the coating or surface opposite the adherent surface becomes nonadherent. The sheet material 11 is now in a condition suitable for handling and cutting as its insulating coating 21 with spacers 22 will not accidentally flake off.

There are several ways of applying a coating with spacers to a sheet material and the following described method is a preferred one. If the sheet material is obtained in large rolls the coating is applied to its top surface as it unrolls by such means as a tank 13 with a spigot containing coating material 12. The unrolled sheet material is then passed between two circumferentially grooved coating rolls 14 which form continuous thin insulating coatings 23 and spacing ridges 22 having a distinctly greater thickness. The roll applying the underneath coating runs immersed in a vat containing the coating material.

The spacing elements 22 may be varied by changing the width, depth and patterns of the grooves in the rolls. A suitable pattern is evenly spaced circumferential grooves 19 of rectangular cross section transversed by another groove 20. Diagonal grooves, holes, spiral grooves, and cross hatched grooves are other suitable patterns within the scope of this invention.

The two coating rolls 14 are set apart at a predetermined distance with a small gap between each roll and the sheet material 11. One roll is placed in near contact above the sheet material and the other roll is placed in near contact underneath the sheet material. As the sheet material 11 containing the coating 12 passes between the grooved rolls 14 an insulating coating 21 comprising alternately arranged low areas 23 and high areas 25 of spacers 22 is formed on the surfaces of the sheet material. The depth of this insulating coating is dependent on the positioning of the rolls 14. Thus, to increase the depth of the coating 21 the rolls 14 are moved farther apart from each other and the sheet material 11.

After being coated the material is passed through an oven 16 which causes the water in the coating solution to evaporate without harming the coating. The resulting insulating and spacing coating 21 adheres to the magnetic material 11 so that it may be freely handled in winding and other forming operations which occur before the 45 final anneal without any substantial amount of the refractory substance rubbing off.

The strip material is then formed into a wound core 17 and placed in the annealing furnace 18. It is essential that the spacers 22 are capable of supporting the 50 weight of the laminations because these laminations frequently become pliable and weakened during high annealing temperatures. During annealing a portion of the insulating coating 21 on the surfaces of the wound core decomposes freeing a portion of coating 22, the freed portion having performed its function as a spacer. Another

portion of the adherent coating 23 reacts with the surface of the steel to form a final and permanent insulating bond. The insulating coating 21 on the surfaces of the wound core decomposes during annealing causing removal of the inert spacers. Thus the core 17 in a single operation is provided with a permanent insulating coating and an easily removable spacer which provides uniform spacing between its laminations and consequently may be rapidly assembled into the electrical coils. Thus, the wound core 17 having been annealed, is stress relieved and because of the spacers 22 has uniform space between its laminations and consequently may be rapidly assembled into the electrical coils.

While only one embodiment of the present invention has been described, it will be apparent to those skilled in the art that other modifications may be employed without departing from the spirit of the invention or from the scope of the appended claims.

#### What is claimed is:

1. A core with laminations of a magnetic sheet material, said sheet material having thereon a coating comprising a composition of a refractory substance and a bonding agent, a surface of said coating adhering to said sheet material and having a nonadherent surface opposite said adherent surface, said nonadherent surface having raised spacing areas for maintaining a spaced relationship between said laminations.

2. A wound core with laminations of a magnetic sheet material, said sheet material having a coating on a plurality of surfaces of said laminations, said coating comprising a composition of a refractory substance and a bonding agent of carboxymethyl hydroxyethyl cellulose, a surface of said coating adhering to said sheet material and having a nonadherent surface removed from said adherent surface, said nonadherent surface having raised spacing areas for supporting said laminations.

#### References Cited in the file of this patent

#### UNITED STATES PATENTS

|           |                 |               |
|-----------|-----------------|---------------|
| 1,454,323 | MacInnes        | May 8, 1923   |
| 2,261,983 | Ford            | Nov. 11, 1941 |
| 2,289,339 | Brennan         | July 14, 1942 |
| 2,389,497 | Gat             | Nov. 20, 1945 |
| 2,390,863 | Amidon et al.   | Dec. 11, 1945 |
| 2,394,047 | Elsey et al.    | Feb. 5, 1946  |
| 2,410,220 | Langworthy      | Oct. 29, 1946 |
| 2,501,349 | Nagel           | Mar. 21, 1950 |
| 2,561,462 | Compton et al.  | July 24, 1951 |
| 2,584,564 | Ellis           | Feb. 5, 1952  |
| 2,655,101 | Newman          | Oct. 13, 1953 |
| 2,670,026 | Ungar           | Feb. 23, 1954 |
| 2,699,195 | Weller          | Jan. 11, 1955 |
| 2,864,065 | Horelick et al. | Dec. 9, 1958  |

#### FOREIGN PATENTS

|         |               |               |
|---------|---------------|---------------|
| 587,374 | Great Britain | Apr. 23, 1947 |
|---------|---------------|---------------|